

# United States Patent [19]

Rentmeester

[11] 3,921,847

[45] Nov. 25, 1975

[54] CEMENTED LAP SEAM CONTAINER

[75] Inventor: Kenneth Richard Rentmeester,  
Barrington, Ill.

[73] Assignee: American Can Company,  
Greenwich, Conn.

[22] Filed: Nov. 7, 1972

[21] Appl. No.: 304,400

|           |         |                        |            |
|-----------|---------|------------------------|------------|
| 3,481,809 | 12/1969 | Kaiser et al.....      | 156/231    |
| 3,524,781 | 8/1970  | Winterroth et al. .... | 156/218    |
| 3,657,380 | 4/1972  | Fang .....             | 117/75     |
| 3,660,194 | 5/1972  | Hoffmann et al. ....   | 156/218    |
| 3,684,617 | 8/1972  | Windecker.....         | 156/330    |
| 3,703,434 | 11/1972 | Schaaf .....           | 117/161 ZB |
| 3,706,619 | 12/1972 | Freeman.....           | 156/330    |
| 3,715,266 | 2/1973  | Winters et al. ....    | 156/330    |
| 3,723,223 | 3/1973  | LeCompte .....         | 156/330    |
| 3,773,589 | 11/1973 | Kaiser et al.....      | 156/330    |

[52] U.S. Cl. .... 220/64; 113/120 A; 220/75;  
220/81; 156/218; 156/309; 156/315;  
156/331; 427/386; 427/388; 427/410;  
428/36; 138/146; 138/151; 138/170; 156/277

[51] Int. Cl.<sup>2</sup> ..... B65D 25/14; B32B 1/08;  
B65D 23/02

[58] Field of Search ..... 156/218, 309, 330, 244,  
156/315, 331, 277; 117/75, 161 ZB; 113/120  
A; 220/62, 75, 64, 81; 138/145, 170, 146,  
151; 161/147, 186; 427/386, 388, 410

[56] References Cited

UNITED STATES PATENTS

|           |         |                      |         |
|-----------|---------|----------------------|---------|
| 2,837,497 | 6/1958  | Delmonte .....       | 156/330 |
| 2,935,488 | 5/1960  | Phillips et al. .... | 260/835 |
| 2,970,077 | 1/1961  | Groves.....          | 156/330 |
| 2,986,546 | 5/1961  | Naps .....           | 156/330 |
| 3,023,189 | 2/1962  | Jupa.....            | 117/75  |
| 3,288,664 | 11/1966 | Hoppe .....          | 156/330 |

Primary Examiner—Douglas J. Drummond

Assistant Examiner—Basil J. Lewris

Attorney, Agent, or Firm—Robert P. Auber; Ernestine  
C. Bartlett; George P. Ziehmer

[57]

ABSTRACT

Can body blanks to be used in production of cemented lap side seam containers are pre-coated with a pigmented epoxy-type coating which, when the body blank is lap side seamed, functions to provide a bonding interface for the lap side seam adhesive while simultaneously functioning as an adherent base upon which to apply printing or other decoration for the exterior surface of the can body thereby permitting elimination of heretofore necessary binding lines and size coat.

25 Claims, 4 Drawing Figures



**FIG. 1****FIG. 2****FIG. 3****FIG. 4**

## CEMENTED LAP SEAM CONTAINER

### BACKGROUND OF THE INVENTION

Cemented, as opposed to soldered, side seam bodies are known in the art. Cans produced from such bodies have found a substantial degree of commercial success for the packaging of products which generate no substantial internal pressure, such as frozen citrus concentrate, household cleaners and polishers, and the like. One of the major selling features of such can bodies is that it is possible to provide printed decorations, as opposed to paper labels, completely around the external surface of a can body. However, such prior art cemented side seam bodies do not have a high degree of bursting strength, particularly when the can is subjected to conditions necessary to process certain products such as the sterilization cooking for fruits and vegetables, or pasturization of beer.

The very high strength adhesives known to the art have not been heretofore successfully used in the manufacture of cemented side seam can bodies for any one of a number of reasons. Some of the major reasons are that although these adhesives have excellent cohesive strength they have been woefully deficient in their adhesion to a metal surface or even to a coating supplied to sheet metal for making can bodies. Another drawback is that these high strength adhesives require a relatively prolonged setting time in the order of minutes or even hours, which time periods are completely unsuitable for high speed can making operations where sufficient bonding strength to hold the can bodies together must be achieved within seconds or less.

Recently, can bodies and methods therefor have been provided which overcome the disadvantages discussed above. Such a procedure, for example, is disclosed in copending application Ser. No. 202,096 filed Nov. 26, 1971 in the names of K. R. Rentmeester and E. W. Kaiser now U.S. Pat. No. 3,773,589 issued Nov. 20, 1973, wherein tubular sheet metal can bodies having opposed longitudinal edges overlapped to form a lap side seam are provided wherein the opposed surfaces of the sheet metal include within the lap side seam an organic coating containing epoxide resin and high-strength organic adhesive disposed within the lap side seam and adhered to the organic coating. As described in said copending application, the coating extends over the entire flat surfaces of the sheet metal and as a result thereof over the entire inside and outside surface of the can body. The coating employed in said copending application also provides an adherent base upon which to apply printing or other decoration for the outside surface of the can body and the decoration is most conveniently applied in the flat, i.e., to that surface of the blank which will later form the outside surface of the can body. Heretofore, the decorative coating has not been permitted to extend into the margin to which the adhesive is to be applied so as to assure that the adhesive would be bonded directly to the coating. Thus, in the procedure of said copending application, as well as in other procedures which do not have the attendant advantages of the procedure of said copending application, it has generally been the procedure in applying decorative coatings to first apply a primer or size coat to protect the metal surface and to provide a bonding interface for the adhesive. A further top coat which may be pigmented, printed or otherwise decorated is then applied but such decorated top coat

has not been permitted to extend into the lap seam. This has been a necessary practice since pigmented or painted surfaces have not been readily bondable. The application of a first "size" or "primer" coat followed by application of a pigmented or decorative coat which is applied to only a portion of a can body blank leads to expense and difficulty. Aside from the care and equipment needed to produce the blank, the top coated or decorated blank contains an unpigmented or undecorated area usually seen as a ragged edge which detracts from the overall aesthetic effect. This area is usually hidden by binding lines. This is an added and expensive operation and detracts from all around lithography and decoration; there is therefore within the can making industry a considerable need for a container, produced by a cemented lap side seam process, which retains the advantages of containers produced by such a process, from a can body blank to which a protective and decorative coating has been applied to the entire exterior surface, which eliminates the need to apply a first size coat followed by a decorative coat followed by application of binding lines.

It is therefore an object of the present invention to provide a lap side seam can body having applied to the exterior surface thereof a pigmented coating which functions to provide a bonding interface for the lap side seam adhesive while simultaneously functioning as a adherent base upon which to apply printing or other decoration to the entire surface.

Another object of the present invention is to provide a lap side seam can body having applied thereto such an exterior pigmented coating and having exceptionally high bursting or hoop strength.

Another object is to provide a lap side seam can body having applied thereto such an exterior pigmented coating and which maintains its high bursting or hoop strength even after it is subjected to prolonged conditions of moist heat.

Yet another object is to provide a decorated lap side seam can body which can be made rapidly on high speed automatic equipment.

A further object is to provide a method for production of a lap side seam can body which eliminates the necessity of applying a first size or prime coat, a decorative top coat and binding lines as in the prior art.

Numerous other objects and advantages of the invention will be apparent as it is better understood from the following description which, taken in connection with the accompanying drawings, discloses the preferred embodiment thereof.

### SUMMARY OF THE INVENTION

The above objects are accomplished by providing a tubular sheet metal, lap side seam can body having as a decorative coating on its entire exterior surface, a baked organic coating containing a pigmented cured epoxide. Preferably, this coating is the heat-cured reaction product formed by applying and baking a coating composition comprising an epoxy resin and a pigment, for example, an epoxy ester and titanium dioxide, the pigment to non-volatile vehicle ratio preferably being about 40-65 parts pigment per 60-35 parts non-volatile vehicle, the opposed coated surfaces being bonded together with a linear superpolyamide adhesive. This can body is formed from a flat blank having at least one entire surface coated in the manner described and having the adhesive applied, before bonding of the lap side seam, to the coating on at least one

of the longitudinal margins thereof. The method and apparatus for making the can body blank is described in U.S. Pat. No. 3,481,809 in the names of Edward William Kaiser, Arnold Robert Rein and Richard Otto Rahler.

Other methods and apparatus for forming the tubular can body and lap side seam as well as for applying the adhesive may be as disclosed in U.S. Pat. No. 3,508,507 issued to A. T. L. Austing and copending U.S. applications Ser. No. 75,530 filed Sept. 25, 1970 in the name of K. R. Rentmeester, now U.S. Pat. No. 3,760,750 issued Sept. 25, 1973 and Ser. No. 79,243 filed Oct. 8, 1970 in the names of K. R. Rentmeester and P. H. Winterroth, now abandoned.

In carrying out the method in accordance with the present invention, the steps of forming the blank into tubular shape, applying the superpolyamide to the longitudinal margin areas, heating the adhesive, and pressing the opposed lap seam surfaces together between chilled supporting surfaces are effected automatically, less than about one second being required for heating the adhesive and pressing the lap seamed surfaces to form the bonded seam.

#### DETAILED DESCRIPTION OF THE INVENTION

Referring to the drawings:

FIG. 1 is a perspective view of a can body blank of the instant invention.

FIG. 2 is a perspective view of a can body of the instant invention;

FIG. 3 is a fragmentary enlarged sectional view taken along line 3—3 of FIG. 2;

and FIG. 4 is a fragmentary enlarged sectional view of a can body of the prior art taken substantially along line 3—3 of FIG. 2.

As the preferred or exemplified embodiment of this invention, FIG. 1 shows a substantially rectangular can body blank generally designated 10 having for the metal component thereof thin guage sheet metal 11 in the order of magnitude of ten thousandths of an inch. This sheet metal, which may be thicker or thinner than the numerical number given, may be aluminum or low carbon steel, with or without an external plating of aluminum, chromium, cobalt, nickel or tin. Completely covering the exposed, extensive exterior flat surface 14 is a particular pigmented and decorative organic coating composition 13 which will be defined more thoroughly hereinafter. Covering the extensive interior flat surface 12 is an organic coating 19 which will be defined more thoroughly hereinafter. Tenaciously adhered to a coating 19 along the inside surface of one longitudinal surface 16 of the blank 10 is an organic cement or adhesive 18, which will also be defined more fully hereinafter. The adhesive 18 extends the full length of the margin 16 and inwardly from the edge of this margin, i.e., has a width of from three thirty-seconds inch to nine thirty-seconds inch and preferably 0.200 inch, and upwardly from the coated surfaces of the margin, i.e., has a thickness of from 0.003 inch to 0.006 inch and preferably about 0.004 inch.

The blank 10 is formed into an open ended tubular can body generally designated 20 (FIG. 2), on a high speed automatic, can body maker, for example of the type utilizing the body-blank applicator of the aforementioned U.S. Pat. No. 3,481,809, bylapping the blank 10 around a mandrel, heating the adhesive 18 to a semi-fluid, tacky condition and pressing onto the coated upper surface or the opposite blank margin 17.

Immediately thereafter the bonded side seam is chilled to set the adhesive and to secure the lapped margins together to form the can body 20 having a lapped side seam generally designated 22, including an inner lap 24 (from the margin 16) and an outer lap 26 (from the margin 17). Bonding of the lapped margins is accomplished in less than one second and preferably in about 10 milliseconds. A container bodymaker which performs this function is described in U.S. Pat. No. 3,508,507 issued to A. T. L. Austing.

As best shown in FIG. 3, the adhesive 18 does not bond directly to the sheet metal 11 of the can body but rather to the opposed surfaces of the exterior organic pigmented epoxy coating 13 and interior coating 19 included within the side seam 22. In other words, the high strength bond of the lap side seam 22 is a result of the tenacious adherence of the coatings 13 and 19 to the sheet metal 11 and to the organic adhesive 18 interposed between the coated faces of the margins 16 and 17.

As stated previously, the coating 13 extends over the entire flat exterior surface 14 of the sheet metal 11 and as a result thereof over the entire outside or exterior surface of can body 20. The coating 13 provides an adherent base upon which to apply printing or other decoration to the surface of the can body as well as a protective coating for the metal over its exposed surface. Decoration (not shown) is more conveniently applied in the flat, i.e., to that surface of the blank 10 or of a larger sheet from which the blank is cut which will later form the outside surface of the can body. As best illustrated in FIG. 3, the decorative coating extends into the bonding area to which the adhesive 18 is subsequently adhered. An appreciation of the present container over the prior art containers may be seen in FIG. 4 wherein a protective coating 25 was first applied over which a decorative top coat 23 was applied. The decorative top coat in FIG. 4 does not extend into the margin 26 to which the adhesive 28 is adhered, since adhesion is effected via bonding of the adhesive to the unpigmented size coating 25.

The coating 13 of this invention, mentioned hereinabove, comprises a pigmented epoxide resin having, before curing, an epoxide equivalent of from 425 to 6,000 and a number average molecular weight of from 1,000 to 4,000 and components coreactive therewith upon application of heat to form an epoxy resin which is preferably an epoxy-ester, epoxy-amino or epoxy-phenolic resin, and such classes of resins modified with various additives such as melamine, urea formaldehyde resins and mixtures thereof.

Any epoxy resin which, when pigmented as in the instant invention, forms a suitable bonding interface and base for receiving decorations may be employed. Epoxy-ester resins, generally derived by reaction of an epoxy-ether having an average molecular weight of about 1,000 to 2,000, and having an epoxide equivalent weight of about 875 to 1,025 with a fatty acid, as for example, saturated and unsaturated fatty acids derived from linseed oil, soya, dehydrated castor oil, tall oil, etc., or simple fatty acids such as oleic, lauric, stearic, palmitic, myristic, linoleic, sorbic, etc. and mixtures thereof may be employed and are especially preferred herein. Epoxy-ester resins are generally obtained by esterifying an epoxy-ether with said acids in relative proportions of about 1 equivalent epoxy to about 0.3 to 0.9 equivalent of fatty acid.

Other suitable epoxy resins are epoxy-amino resins, derived by reaction of epoxy-ethers having an average molecular weight, before curing, of about 900 to about 4,000 with various amino-containing resins such as melamine, triazine, ureaformaldehyde, etc. Such epoxy amino resins are generally obtained via reaction of epoxy ethers, for example, diglycidyl ether of bisphenol A with such amino-containing resins in relative proportions varying from about 95/5 to 50/50. Other suitable epoxy resins include epoxy-phenolic resins which include reaction products of various polyhydric phenols for example, allyl ether of polymethylol phenol, polymethylol tertiary butyl phenol, polymethylol p-phenylphenol, etc., with epichlorohydrin and similar epoxidic materials by methods known in the art. Suitable epoxides of this class will have, before curing, an epoxide equivalent of about 425 to 6,000 and an average molecular weight of about 1,000 to 4,000 and include polyglycidyl ethers of bisphenol A, epoxidized novolacs, etc.

Thus, the epoxy-ester, epoxy-amino and epoxy-phenolic resins suitable for use in the invention are well known in the art and may be prepared by incorporation of the reacting components in the formulation including catalysts and modifying agents as desired. Particularly preferred are such resins modified through further reaction with melamine, ureaformaldehyde resins and combinations thereof. The epoxy resins, as employed herein, are pigmented with proportions of pigment to non-volatile vehicle being generally within the range of about 40 to 65, preferably 50 to 60, parts by weight of pigment to 60 to 35, preferably 50-40, parts of non-volatile vehicle. Exemplary of suitable pigments are titanium dioxide, colloidal silica, zinc oxide, and aluminum pastes or powders. Both rutile and anatase forms of titanium dioxide are preferred for use herein with rutile titanium dioxide being especially preferred.

Extender pigments may be employed where desired. In general, however, such ingredients are not employed particularly in formulating white coatings which are applied as relatively thin films and any substantial use of extenders would tend to detract from the desired coverage and aesthetic quality of the coating. Where it is desired to employ such extenders, however, conventional extender pigments known in the art, for example, calcium carbonate, may prove suitable. Various other additives such as flow control agents, suspending aids, and compatible lubricants may be employed as desired. The coating 13 is preferably applied as a dispersion of the above described ingredients, before their interaction, in a fugitive liquid. It is necessary that the liquid be volatile at baking temperatures which may be as low as 300°F. or as high as 650°F. At the lower temperature, a baking period of about 10 minutes may be required and at the upper temperature a time of five seconds may suffice. The solvent must also be compatible with all the ingredients in their useful concentrations, so that precipitation, stratification or other separation does not occur. Suitable solvents comprise aryl or aralkyl hydrocarbons blended with alcohols, ketones, ethers or esters and mixtures thereof. Alcohol, ketones, ethers or esters or mixtures thereof may be employed without aryl or aralkyl hydrocarbons if desired. Solvent systems comprising a mixture of aryl or aralkyl hydrocarbons and alcohols yield solutions having optimum viscosity for application and for this reason are preferred.

Examples of the aromatic hydrocarbons solvents are xylene, toluene, and petroleum fractions having a high proportion of aromatic hydrocarbons and having a boiling range of about 230°F. to 415°F. Examples of suitable oxygen containing solvents are butanol, diacetone alcohol, isophorone, methylisobutylketone, nitropropane, ethylene glycol monobutyl ether, tetrahydrofuran, cyclohexanone, amyl acetate, ethylene glycol monomethyl ether acetate, diisobutyl ketone and cyclohexanone.

In the specific example which follows, the first three ingredients were dissolved in the remaining solvent components and uniformly applied to one large flat surface of sheet aluminum. The thus coated sheet was passed into an oven and baked under the conditions of temperature and time above discussed and thereafter cooled. Subsequently, the coating is printed as desired and preferably varnished over the printed label to provide the decorative coating 13.

After application of the fluid coating composition described immediately below and during the baking of the thus coated sheet described hereinafter, the non-volatile ingredients are inter-reacted and the volatile organic liquid is driven off so that upon completion of the baking operation and subsequent cooling, the solid inert adherent coating 13 remains on the metal sheet 11. A specific example of a fluid composition for application to the metal sheet 11 to provide the finished coating is as follows:

| MATERIAL                                                                            | PARTS BY WEIGHT |
|-------------------------------------------------------------------------------------|-----------------|
| Epoxy Resin (A glycidyl ether of bis Phenol A having an average M.W. of about 2900) | 19.0            |
| Urea-Formaldehyde Resin (Rohm & Haas 3300) (50% total solids)                       | 12.3            |
| Titanium Dioxide Pigment (Dupont R110)                                              | 19.7            |
| Diacetone Alcohol                                                                   | 14.7            |
| Diisobutyl Ketone                                                                   | 4.9             |
| Isophorone                                                                          | 4.9             |
| Xylene                                                                              | 17.1            |
| n-Butanol                                                                           | 7.4             |
|                                                                                     | 100.0           |

In addition to the above described exterior coating, epoxy based coatings may be employed to form interior coatings 19 for the interior surfaces 12 of the container body. Such coatings may be unpigmented or pigmented epoxy resins as described above, or may include any of well known coatings employed for this purpose. One such other coating which may be employed is an epoxy-urea-formaldehyde coating wherein the epoxy component is a 1, 2-epoxide resin substantially similar to the epoxy-ethers hereinbefore described. Historically, it has been preferred that the inside coat for beverage containers be of some color. This preference has more significance in lap seam cemented cans because a coating must also be applied to the exterior surface in order to do the cementing job. Such a colored inside coating is desirable since it is often desired to have a difference in color between the inside and the outside of a container body, so that the printing press man can immediately determine if he is printing on the correct side of the sheet. For this reason it is preferred that the can body blank be coated on the surface that is to form the interior of a container body with an epoxy resin having a pigment different from that applied to the exterior surfaces, for example, a gold tartrazine lake pigment.

Additionally, the decorative, pigmented epoxy exterior coating may, if desired, be coated with a further clear varnish for protection of the decorative label once it has been applied. Such varnishes may be conventional lacquers such as alkyds, acrylics, etc. It will be understood, however, that such additional coating is not mandatory nor is it limited to the specific examples above enumerated and may include any of conventional coatings known in the art.

The linear superpolyamide adhesives useful in the instant invention are generally characterized by having recurring aliphatic amido groups separated by alkylene groups having at least two carbon atoms and having an inherent viscosity of at least 0.4. These superpolyamides are disclosed in U.S. Pat. Nos. 3,256,304; 10 2,962,468; 3,397,816; 3,447,999; 3,249,629, etc.

As employed herein, inherent viscosity  $\eta_{inh}$  is defined by the following equation:

$$\eta_{inh} = \frac{\ln \eta_{rel}}{C}$$

wherein  $\ln \eta_{rel}$  represents the natural logarithm of the relative viscosity and

$$\eta_{rel} = \frac{\eta_{\text{solution}}}{\eta_{\text{solvent}}}$$

$\eta$  being viscosity and C the concentration of the solute in grams per 100 cc. of solution. The inherent viscosity values employed herein are obtained with the polyamide involved dissolved in m-cresol at a concentration of 0.5 g. of polymer per 100 cc. of solution at 25° C.

Among the superpolyamides which are useful in the present invention and having inherent viscosities as described above are polypentamethylene sebacamide, polyhexamethylene adipamide, polyhexamethylene sebacamide, poly-m-phenylene sebacamide, 6-amino-caproic acid polymers, 7-amino-heptanoic acid polymers, 11-amino undecanoic acid polymers, and 12-amino-stearic acid polymers; polyamides derived from reaction of polymeric fat acids with various amines for example polyamides derived from polymerized tall oil, 10-undecynoic, soybean, dehydrated castor oil, cottonseed, linoleic, etc., acids and organic diamines, triamines, tetramines, etc., as described in the above-identified patents, the disclosures thereof being incorporated herein by the foregoing references thereto.

It is thought that the new invention and many of its attendant advantages will be understood from the foregoing description and it will be apparent that various changes may be made in the matter of ingredients, the identity and the proportions of formulation, and that changes may be made in the form, construction and arrangement of the parts of the article without departing from the spirit and scope of the invention of sacrificing all of its material advantages, the form hereinbefore described being merely a preferred embodiment thereof.

I claim:

1. A decorated, tubular, sheet metal can body having opposed longitudinal edges overlapped to form a lap side seam wherein the interior metal surface within the seam is adjacent to and overlaps the opposed exterior metal surface within the seam, the opposed surfaces included within said lap seam having adhered thereto an

5 organic coating comprising an epoxy resin, and an organic adhesive disposed in said lap seam and adhered to the coating on said surfaces, said organic adhesive being a linear superpolyamide having an inherent viscosity of at least 0.4;

10 the coating on the entire exterior surface being a cured, decorative pigmented organic coating which extends into the lap seam, constitutes a bonding interface for the organic adhesive and an adherent base receptive to printing or other decoration, said cured coating being derived from a composition comprising from about 40 to about 65 parts by weight of a pigment and from about 60 to about 35 parts by weight of non-volatile vehicle comprising an epoxy ether having, before curing, an epoxide equivalent of from 425 to 6,000 and a number average molecular weight of from 1,000 to 4,000 and components coreactive therewith upon application of heat to form an epoxy resin, the epoxy resin thus formed being selected from the group consisting of (1) epoxy-phenolic (2) epoxy-ester and (3) epoxy-amino resins.

2. A decorated, tubular, sheet metal can body as defined in claim 1 in which said coating on the exterior surface comprises an epoxy-ester resin derived from the reaction of a diglycidyl ether of bisphenol A and oleic acid.

25 3. A decorated, tubular, sheet metal can body as defined in claim 1 in which said coating on the exterior surface comprises an epoxy-amino resin derived from the reaction of a diglycidyl ether of bisphenol A and a ureaformaldehyde resin.

30 4. A decorated, tubular, sheet metal can body as defined in claim 1 in which said coating on the exterior surface comprises an epoxy-phenolic resin derived from the reaction of a diglycidyl ether of bisphenol A and a polyhydric phenol.

45 5. A decorated tubular sheet metal can body as defined in claim 1 in which said pigment is titanium dioxide.

60 6. A decorated, tubular, sheet metal can body as defined in claim 1 in which said coating on the exterior surface comprises an epoxy-ester resin derived from reaction of a diglycidyl ether of bisphenol A having an average molecular weight of about 1400 and oleic acid, said adhesive is a linear superpolyamide having recurring aliphatic amido groups separated by alkylene groups having at least two carbon atoms and said pigment is titanium dioxide.

50 7. A decorated, tubular sheet metal can body as defined in claim 1 in which the pigmented coating on the exterior surface is printed.

55 8. A method of fabricating a decorated, tubular, metal can body having its opposed longitudinal edges overlapped to form a lap side seam comprising:

65 applying to the entire exterior surface of the sheet metal to be formed into a can body, a decorative pigmented organic coating formulation comprising, as the non-volatile vehicle, about 60 to about 35 parts by weight of an epoxide having before curing, an epoxide equivalent of from 425 to 6,000 and a number average molecular weight of from 1,000 to 4,000 and components coreactive therewith upon application of heat to form an epoxy resin, the epoxy resin thus formed being selected from the group consisting of (1) epoxy-phenolic (2) epoxy-ester and (3) epoxy-amino resins, and about 40 to about 65 parts by weight of a pigment,

said pigmented coating constituting a bonding interface for a lap side seam adhesive and an adherent base receptive to printing or other decoration; baking the coated sheet metal at a temperature of at least 300°F, to cure the organic coating thereon; forming said coated sheet metal into a tubular can body, arranged to have a lap side seam wherein the interior metal surface within the finished seam is adjacent to and overlaps the opposed exterior metal surface within the seam, there being applied to at least one of said opposed surfaces forming the seam an organic adhesive comprising a linear superpolyamide having an inherent viscosity of at least 0.4;

and bonding said opposed surfaces to form the finished seam, said decorative pigmented coating extending into the lap seam thus produced.

9. A method as claimed in claim 1 wherein said cured epoxide is an epoxy-ester resin.

10. The method of claim 9 wherein said pigment is titanium dioxide and said epoxy ester resin is the reaction product of an epoxy-ether and a fatty acid.

11. The method of claim 10 wherein said fatty acid is oleic acid.

12. The method of claim 11 wherein said formulation consists of 50 - 60 parts titanium dioxide to 50 - 40 parts non-volatile vehicle.

13. A method as claimed in claim 1 wherein said cured epoxide is an epoxy-amino resin.

14. A method as claimed in claim 1 wherein said cured epoxide is an epoxy phenolic resin.

15. A method as claimed in claim 1 wherein said coating contains a urea-formaldehyde resin.

16. A method as claimed in claim 1 wherein said organic adhesive applied within the seam is a linear superpolyamide having recurring aliphatic amido groups separated by alkylene groups having at least two carbon atoms.

17. A method as claimed in claim 1 wherein said steps of applying said organic adhesive, forming said tubular shape, and bonding are carried out automatically, said step of bonding the opposed surfaces being effected in less than about 1 second.

18. A method as claimed in claim 1 wherein the surface of the sheet metal which is to form the interior surface of the can body is coated with a 1, 2-epoxide resin.

19. A method as claimed in claim 1 wherein said pigment is titanium dioxide.

20. A method as claimed in claim 1 wherein said coated sheet is printed prior to forming into said tubular can body.

21. A method of fabricating a decorated, tubular, sheet metal can body having its opposed longitudinal edges overlapped to form a lap side seam, comprising:

applying to the interior surface of the sheet metal to be formed into a can body an organic coating comprising a 1,2-epoxide resin having before curing an epoxide equivalent of from about 425 to 6,000 and a number average molecular weight of from 1,000 to 4,000;

10  
5  
10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
86

UNITED STATES PATENT OFFICE  
CERTIFICATE OF CORRECTION

PATENT NO. : 3,921,847

DATED : 11/25/75

INVENTOR(S) : Kenneth Richard Rentmeester

It is certified that error appears in the above-identified patent and that said Letters Patent are hereby corrected as shown below:

In the Specification:

At col. 3, line 68, change "or" to ---of---.

At col. 5, line 47, delete the semi-colon after carbonate and substitute a comma therefor.

In the Claims:

In line 1 of each of claims 9, 13, 14, 15, 16, 17, 18, 19 and 20, change "1" to --8--.

In line 1 of each of claims 22, 23 and 24, change "14" to --21--.

Signed and Sealed this  
second Day of March 1976

[SEAL]

Attest:

RUTH C. MASON  
Attesting Officer

C. MARSHALL DANN  
Commissioner of Patents and Trademarks